

# United States Patent Office

2,860,107

Patented Nov. 11, 1958

1

2,860,107

## CONTROLLED SUDSING HEAVY DUTY LIQUID DETERGENT

Vincent Lamberti, Hackensack, and Arthur O. Gray, Jr., River Edge, N. J., assignors to Lever Brothers Company, New York, N. Y., a corporation of Maine

No Drawing. Application July 25, 1957  
Serial No. 674,048

4 Claims. (Cl. 252—137)

The present invention relates to detergent compositions, and more particularly to controlled sudsing heavy duty liquid detergent compositions which have phase stability on storage.

Many detergent compositions have heretofore been prepared, but they have primarily been in a powdered form and thereby have many disadvantages enumerated below. Powdered detergent compositions are generally prepared by spray drying or drum drying, which are costly operations. When used in washing, the powdered detergent compositions must be dissolved to form dilute aqueous washing solutions. This step of dissolving or dispersing the powdered detergent compositions in the wash water is time consuming. Frequently, the powdered detergent compositions are difficultly dispersed, since they may tend to form lumps. Powdered detergent compositions, moreover, tend to vary greatly in density unless particular care is taken in their preparation. Such a variation in density makes it difficult to determine the exact amount thereof to be employed during washing. In addition, powdered detergent compositions may be difficult to dispense, since they sometimes clog the orifices of a dispenser. Also powdered detergent compositions have a tendency to cake at high humidities upon standing in their own containers. Moreover, powdered detergent compositions, being normally sold in cardboard containers, are subject to spilling and waste in the event an open container is accidentally knocked over. Furthermore, their dustiness may be bothersome, particularly to persons who suffer from dust allergies.

All of these disadvantages of powdered detergent compositions can be obviated by employing concentrated liquid detergent compositions. While light duty liquid detergent compositions have been prepared heretofore, they have proved to be suitable only for dishwashing and the cleaning of fine fabrics. Light duty liquid detergent compositions are unsatisfactory for washing heavily soiled cotton fabrics, since such compositions have inadequate soil removal characteristics. Heavy duty liquid detergent compositions, on the other hand, have excellent soil removal characteristics and are ideally suited for the washing of heavily soiled cotton fabrics and other fabrics.

A heavy duty liquid detergent must be homogeneous in composition at the time of addition to the washing machine in order to insure that the washing solution will contain the proper ratio of ingredients. The consumer buys a detergent product after it has been subjected to various temperatures and conditions of storage between the time of production and arrival on the dealers' shelves. These various storage conditions have greater adverse effect on a liquid product containing a delicately balanced active detergent and cellulosic suspension than on a detergent powder.

A heavy duty liquid detergent designed for use in both horizontal (front loading) and upright (top loading) washing machines must have acceptable sudsing and

2

detergent properties when used in either of these machines. When high sudsing detergent products are used in front loading horizontal tumbler type automatic washers, these products foam profusely causing the tumbler to fill or overflow with dense suds. These dense suds impede the washing action by interfering with the free fall of clothes in the tumbler and may strain the working parts of the machine to cause slowing or stalling, further impeding washing action, and causing excessive wear of machine parts. When using high sudsers in this type of washer, the housewife is inclined to reduce usage level in order to eliminate this excess sudsing. The amount of product thus used is frequently insufficient to wash effectively or to provide the desired level of optical brightener.

Profuse sudsing in top loading vertical agitator-type automatic washers does not interfere with washing action, but may tend to cause suds-lock during the extraction cycle. Suds-lock prevents efficient extraction of water from the clothes by slowing or stalling the machine, and also causes excessive wear of machine parts.

A low-sudsing detergent product will produce no suds coverage when used in an upright washing machine. This lack of suds coverage does not obscure the dirty water from view and leads to the impression that too little product was used. The consumer may add more product in an attempt to obtain suds coverage. Such overuse of the product is uneconomical and may be reflected in failure of the consumer to repurchase.

Accordingly, it is an object of the present invention to provide heavy duty liquid detergent compositions which have controlled suds, i. e., there is neither a high amount nor a low amount of suds, but rather a medium amount of suds. It is a further object of the invention to provide heavy duty liquid detergent compositions in which the amount of suds produced therefrom is stable over a relatively prolonged period, especially in the presence of soil. It is also an object of the invention to provide heavy duty liquid detergent compositions which have phase stability, i. e., there is a minimum of separation of the various components therein upon storage.

The above objects have been accomplished by formulating heavy duty liquid detergent compositions having various critical factors which include the number of the components making up the compositions, the nature of the components present therein, and the amounts of the components utilized therein. The compositions of the invention consist essentially of aqueous suspensions of various components as further identified below.

The compositions contain as an active detergent component potassium dodecylbenzene sulfonate in an amount from about 2% to about 3%. The potassium dodecylbenzene sulfonate supplies a portion of the foaming and wetting action necessary in a heavy duty liquid detergent product designed for household use. This component may be added to the compositions as dodecylbenzene sulfonic acid which is converted in situ by potassium hydroxide used to adjust the pH of the compositions.

The compositions also contain as a further active detergent component from about 3.5% to about 5% of sodium tallow methyl taurate. This component is derived from the naturally occurring mixture of fatty acids present in tallow.

A further component of the heavy duty liquid detergent compositions is tetrapotassium pyrophosphate. This component which is used in an amount from about 22.5% to about 25% supplies the heavy duty detergent feature of the liquid and imparts good soil removal properties thereto.

The compositions also contain from about 2% to about 3% of an alkali metal xylene sulfonate, such as sodium xylene sulfonate or potassium xylene sulfonate.

The xylene sulfonate acts as a hydrotrope in solubilizing the active detergent components of the compositions in the presence of a considerable amount of the polyphosphate and any other inorganic materials.

There is also present in the compositions about 1% of coconut oil fatty acids, i. e., the naturally occurring mixture of fatty acids present in coconut oil, as well as about 1% of the condensation product of one mole of lauric monoethanolamide with one mole of ethylene oxide, and about 1% of triethanolamine. These components together aid in imparting phase stability and suds stability to the heavy duty liquid detergent compositions.

The compositions of the invention also contain a pair of cellulosic soil suspending agents which form a uniform, stable suspension therein even under adverse storage conditions. This pair of cellulosic soil suspending agents consists of about 0.3% of sodium carboxymethylcellulose and about 0.7% of Methocel. The sodium carboxymethylcellulose contains 0.7 mole of carboxymethyl groups per anhydroglucose unit. Methocel is a trade name for methylcellulose of 25 centipoise viscosity in a

acids, the condensation product of one mole of lauric monoethanolamide with one mole of ethylene oxide, the triethanolamine, and any optical brighteners, and tetrapotassium pyrophosphate. The compositions are completed by the adjustment with alkali to a pH of about 12 followed by the addition of the alkali metal silicates.

The controlled sudsing heavy duty liquid detergent compositions of the invention having phase stability on storage and suds stability on usage will be further illustrated by the following examples.

The compositions of the invention were prepared as were other compositions in which various components of the compositions of the invention were omitted in order to demonstrate forcefully the criticality of the presence of the various components in the compositions. These compositions are set forth below in Table I wherein Compositions X, X', and X'' are the compositions of the invention containing various optional components, namely sodium silicate, potassium hydroxide, and fluorescent dye, while Compositions A through F are comparative compositions wherein various components of the compositions of the invention were omitted.

TABLE I

| Components                                                                                      | Compositions (Percent by Weight) |        |        |       |       |       |       |       |       |
|-------------------------------------------------------------------------------------------------|----------------------------------|--------|--------|-------|-------|-------|-------|-------|-------|
|                                                                                                 | X                                | X'     | X''    | A     | B     | C     | D     | E     | F     |
| Dodecylbenzene Sulfonic Acid                                                                    | 2.04                             | 2.816  | 2.816  | 5.65  |       | 2.04  | 2.04  | 2.04  | 2.04  |
| Sodium Tallow Methyltaurate                                                                     | 3.61                             | 5.0    | 5.0    |       | 5.65  | 3.61  | 3.61  | 3.61  | 3.61  |
| Sodium Xylene Sulfonate                                                                         | 2.17                             | 3.0    | 3.0    | 2.17  | 2.17  | 2.17  | 2.17  | 2.17  | 2.17  |
| Coconut Oil Fatty Acids                                                                         | 1.0                              | 1.0    | 1.0    | 1.0   | 1.0   |       | 1.0   |       |       |
| The Condensation Product of One Mole of Lauric Monoethanolamide with One Mole of Ethylene Oxide |                                  |        |        |       |       |       |       |       |       |
| Triethanolamine                                                                                 | 1.0                              | 1.0    | 1.0    | 1.0   | 1.0   |       |       |       | 1.0   |
| Sodium Carboxymethylcellulose (as identified above)                                             | 1.0                              | 1.0    | 1.0    | 1.0   | 1.0   |       |       |       |       |
| Methocel (as identified above)                                                                  | 0.25                             | 0.25   | 0.25   | 0.25  | 0.25  | 0.25  | 0.25  | 0.25  | 0.25  |
| Tetrapotassium Pyrophosphate                                                                    | 0.68                             | 0.68   | 0.68   | 0.68  | 0.68  | 0.68  | 0.68  | 0.68  | 0.68  |
| Sodium Silicate ( $\text{Na}_2\text{O} \cdot \text{SiO}_2$ of 1:2.5)                            | 25.0                             | 25.0   | 25.0   | 25.0  | 25.0  | 25.0  | 25.0  | 25.0  | 25.0  |
| Fluorescent Dye (Uvitex SI)                                                                     | 3.1                              | 2.8    | 3.1    | 3.1   | 3.1   | 3.1   | 3.1   | 3.1   | 3.1   |
| Fluorescent Dye (1:1 mixture of UVITEX SI and Calcifluor White MR)                              |                                  | 0.045  |        |       |       |       |       |       |       |
| Water, Miscellaneous Salts, and Potassium Hydroxide to pH 11.8                                  |                                  |        | 0.09   |       |       |       |       |       |       |
|                                                                                                 | 60.15                            | 59.909 | 57.064 | 60.15 | 60.15 | 63.15 | 62.15 | 62.15 | 62.15 |

2% aqueous dispersion having 27.5-32% methoxyl groups per cellulose molecule.

The remaining essential component of the heavy duty liquid detergent compositions is water which serves as a solvent for the soluble components thereof.

If desired, the heavy duty liquid detergent compositions may contain minor portions of an alkali, such as potassium hydroxide, to neutralize any excess acid impurities present in the components of the compositions. In addition, minor portions of compatible perfumes, fluorescent dyes, optical brighteners, alkali metal silicates, and other desirable adjutants may be added to the compositions. When a water-soluble alkali metal silicate is added to the compositions, the pH thereof must be adjusted to about 12 by the addition of free alkali, such as potassium hydroxide, to keep the silicate in solution. Typical alkali metal silicates include the sodium or potassium silicates having the following alkali to silica ratios: 1:3.92, 1:3.44, 1:3.25, 1:2.5, 1:2.4, 1:2.0, 1:1.8, and 1:1. Generally, about 3% of the alkali metal silicate is employed. The amount of perfumes, fluorescent dyes, and optical brighteners, is quite small and generally is about 0.1% or less.

The controlled sudsing heavy duty liquid detergent compositions of the invention may be prepared by mixing the components thereof together in the aqueous medium. Heat may be conveniently utilized during the mixing of the components to increase the rate of dissolution thereof. A preferred method for the preparation of the compositions is the addition of the pair of cellulosic soil suspending agents to hot water followed by cooling to form an aqueous suspension thereof and the addition to the cellulosic suspension of an aqueous solution of the potassium dodecylbenzene sulfonate, the alkali metal xylene sulfonate, the sodium tallow methyl taurate, the coconut oil fatty

1

Compositions X, X', and X'' of the invention as well as various comparative compositions were tested for phase stability under various conditions of storage. All of the formulations were stored for seven days at various storage temperatures, namely 14° F., 35° F., room temperature (70° F.), and 125° F. In addition, samples of the formulations were subjected to five daily cyclings from 14° F. to room temperature and from 35° F. to room temperature. After undergoing storage the samples were either unaffected, showed a rise or drop of cellulosics, or an uneven cellulosic distribution, or exhibited organic phase separation. In order to facilitate comparison of various formulations the following numerical rating system was used:

| Condition of sample after storage: | Numerical rates |
|------------------------------------|-----------------|
| Satisfactory                       | 0               |
| Very slight rise or drop           | 0.1             |
| Slight rise or drop                | 0.2             |
| 1/16 rise or drop                  | 0.5             |
| Uneven cellulosics                 | 0.5             |
| 1/8 rise or drop                   | 0.5             |
| 1/4 to 1/8 rise or drop            | 1.0             |
| 1/4 rise or drop                   | 1.5             |
| 1/2 rise or drop                   | 2.0             |
| 2/3 rise or drop                   | 3.0             |
| 40% rise or drop                   | 4.0             |
| 50% rise or drop                   | 5.0             |
| 60% rise or drop                   | 6.0             |
| Organic separation                 | 6.0             |

In the above numerical rating system rise or drop refers to the rise or drop of the cellulosic soil suspending agents. In any combination of conditions, the numerical rating numbers are additive, i. e., very slight drop plus uneven

cellulosics equals 0.1 plus 0.5, or a total rating of 0.6. However, the maximum numerical rating in any one condition will be 6.0. The numerical rating for each of the tests conducted were added to give a total rating. Of course, the lower the total rating, the better is the phase stability of the composition.

Data on this phase stability test wherein Compositions X, X', and X'' of the invention were compared with Compositions A through F as typical comparative compositions are set forth below in Table II.

TABLE II  
*Phase stability test conditions and ratings*

| Compositions | 14° F. | 35° F. | Room Temperature | 125° F. | Cycled                     |                            | Total Rating |
|--------------|--------|--------|------------------|---------|----------------------------|----------------------------|--------------|
|              |        |        |                  |         | 35° F. to Room Temperature | 14° F. to Room Temperature |              |
| X            | 0      | 0      | 0.2              | 2       | 0                          | 1.5                        | 3.7          |
| X'           | 0.2    | 0.1    | 0.2              | 1.0     | 0                          | 0.1                        | 1.6          |
| X''          | 0.1    | 0.1    | 0.1              | 0.2     | 0.1                        | 0.1                        | 0.7          |
| A            | 6      | 6      | 6                | 6       | 6                          | 6                          | 36.0         |
| B            | 4      | 4      | 5                | 0.2     | 5                          | 5                          | 23.2         |
| C            | 3      | 0.5    | 0                | 0.1     | 0.2                        | 1                          | 4.8          |
| D            | 3      | 0      | 1.5              | 2       | 1                          | 3                          | 10.5         |
| E            | 5      | 0.5    | 1.5              | 0       | 1.5                        | 5                          | 13.5         |
| F            | 1.5    | 0      | 0                | 0.5     | 0                          | 0.2                        | 2.2          |

From the data set forth above in Table II it will be noted that Compositions X, X', and X'' of the invention had lower total ratings, and hence better phase stability, than did any of the comparative compositions with the exception of Composition X versus Composition F. Composition F, however, does not have the requisite suds stability in water containing soil as shown below in Table III and hence it does not have the balanced properties of both phase stability and suds stability that are possessed by Compositions X, X', and X'' of the invention.

When various other components of the compositions of the invention were omitted therefrom, unstable compositions were also obtained. The phase stability test was also run for compositions containing both less and more of the tetrapotassium pyrophosphates, i. e., 20% and 30% thereof, and more and less of the detergent actives, i. e., potassium dodecylbenzene sulfonate and sodium tallow methyl taurate. These phase stability tests showed that such heavy duty liquid detergent compositions were unstable and accordingly demonstrate the criticality as to the amount of these components which must be employed therein.

Not only are the total number of components present in the compositions critical as well as the amounts thereof, but also the nature of the components is quite critical. Thus, various anionic and nonionic synthetic organic non-soap detergents were substituted for an equal amount of the sodium tallow methyl taurate component of the compositions and phase stability tests run thereon. When each of the following exemplary synthetic detergents was so substituted, the resulting formulations were unstable as determined by the above phase stability test: potassium pentadecylbenzene sulfonate, Santomerse E (a mixture of potassium pentylbenzene sulfonate and potassium hexylbenzene sulfonate), sodium lauryl sulfate, sodium N-ethyl-N-palmitoyl taurate, sodium N-isopropyl-N-hexadecanoyl taurate, sodium N-methyl-N-oleyl taurate, the condensate of dodecyl phenol with 13 moles of ethylene oxide, the condensate of propylene oxide with ethylene oxide, sodium isopropyl naphthalene sulfonate, disodium N-octadecyl sulfosuccinate, potassium  $\alpha$ -sulfopalmitate.

The presence of sodium xylene sulfonate in the controlled sudsing heavy duty liquid detergent compositions of the invention is quite critical, since the substitution therefor of sodium toluene sulfonate or sodium benzene sulfonate produced formulations having poor phase

stability. Moreover, the presence of tetrapotassium pyrophosphate is quite critical, since the substitution of pentapotassium tripolyphosphate therefor produces compositions in which the cellulosic soil suspending agents are unstable and may cause the precipitation of silica from the compositions due to hydrolysis of this polyphosphate.

The suds stability of the controlled sudsing heavy duty liquid detergent compositions of the invention was also tested and compared with other formulations which

omitted various components of the compositions to show the criticality of the components in the compositions of the invention. In the suds stability tests, 0.25 gram of the detergent compositions were each added separately to 100 ml. of water in 500 ml. glass stopped graduated cylinders. Each cylinder was inverted twenty times (10 cycles from upright to upright). Initial suds volume and suds volume at 15 minute intervals for 45 minutes were recorded. Tests were run in distilled water at 120° F. Since the compositions of the invention would normally be used in automatic washers in which the water would contain soil, one drop of Wesson Oil was added. The formulations tested were Composition X of the invention as well as Compositions A through F set forth above in Table I. The data on this suds stability test are set forth below in Table III.

TABLE III

| Time Interval (minutes) | Suds Volume of Compositions (milliliters) |     |     |     |     |     |     |
|-------------------------|-------------------------------------------|-----|-----|-----|-----|-----|-----|
|                         | X                                         | A   | B   | C   | D   | E   | F   |
| 0.....                  | 250                                       | 220 | 200 | 210 | 160 | 125 | 210 |
| 15.....                 | 240                                       | 180 | 180 | 190 | 110 | 115 | 180 |
| 30.....                 | 240                                       | 150 | 85  | 40  | 90  | 100 | 175 |
| 45.....                 | 240                                       | 120 | 70  | 35  | 80  | 50  | 175 |

The data set forth in Table III above clearly show that representative Composition X of the invention had far greater suds stability than did Compositions A through F in view of the small comparative decrease in suds volume over a 45 minute interval. It will be appreciated that the compositions of the invention are concerned with a system of suds which are controlled to a lower level than is desired for non-automatic washers, so that the importance of the data set forth above in Table III lies not in a comparison of the total suds volume, but rather in a comparison of the suds stability or change in suds volume over a period of time.

The controlled nature of the suds produced by the compositions of the invention is evident from the following data in Table IV below wherein 2.6 ounces of Compositions X, X', and X'' were separately added to 8 gallons of water containing soil and the height of suds on the port of a horizontal or front loading Bendix washer observed at 3, 6, 9 and 12 minutes during the washing cycle. In this table the fractions refer to the portion of the port covered by the suds.

7  
TABLE IV

| Compositions | Suds Volume |     |     |     |
|--------------|-------------|-----|-----|-----|
|              | 3'          | 6'  | 9'  | 12' |
| X            | 1/3         | 1/6 | 1/9 | 2/9 |
| X'           | 1/2         | 1/4 | 2/9 | 1/4 |
| X''          | 1/2         | 1/2 | 2/3 | 1   |

When high sudsing detergents were similarly tested, they produced a profuse amount of suds at the end of only three minutes which completely covered the port of the washer.

In view of the above data it will be apparent that the compositions of the invention provide for the first time heavy duty liquid detergent compositions which have phase stability on storage and suds stability in usage and thereby make them products ideally suited for use in automatic clothes washers. Moreover, the controlled sudsing products do not produce excess suds when used in horizontal washing machines, but they do give a showing of suds on the water surface when used in vertical type machines.

It will be appreciated that various modifications and changes may be made in the compositions of the invention without departing from the spirit thereof and accordingly the invention is to be limited only within the scope of the appended claims.

We claim:

1. A controlled sudsing heavy duty liquid detergent composition which has phase stability on storage and suds stability in usage consisting essentially of an aqueous suspension of from about 2% to about 3% of potassium dodecylbenzene sulfonate, from about 3.5% to about 5% of sodium tallow methyl taurate, from about 2% to about 3% of an alkali metal xylene sulfonate, about 1% of coconut oil fatty acids, about 1% of the

condensation product of one mole of lauric monoethanolamide with one mole of ethylene oxide, about 1% of triethanolamine, about 0.3% of sodium carboxymethylcellulose, about 0.7% of methylcellulose, and from about 22.5% to about 25% of tetrapotassium pyrophosphate.

2. A controlled sudsing heavy duty liquid detergent composition which has phase stability on storage and suds stability in usage consisting essentially of an aqueous suspension of about 2% of potassium dodecylbenzene sulfonate, about 3.5% of sodium tallow methyl taurate, about 2% of sodium xylene sulfonate, about 1% of coconut oil fatty acids, about 1% of the condensation product of one mole of lauric monoethanolamide with one mole of ethylene oxide, about 1% of triethanolamine, about 0.3% of sodium carboxymethylcellulose having 0.7 mole of carboxymethyl groups per anhydroglucosidic unit, about 0.7% of methylcellulose of 25 centipoise viscosity in a 2% aqueous dispersion having 27.5-32% methoxyl groups per cellulose molecule, and about 25% of tetrapotassium pyrophosphate.

3. A composition as set forth in claim 2 containing about 3% of an alkali metal silicate and having a pH of about 12.

4. A composition as set forth in claim 2 having a pH of about 12.

#### References Cited in the file of this patent

##### UNITED STATES PATENTS

|            |         |               |
|------------|---------|---------------|
| Re. 23,840 | Vitale  | June 15, 1954 |
| 2,002,613  | Orthner | May 28, 1935  |
| 2,581,677  | Machlis | Jan. 8, 1952  |
| 2,618,607  | Sanders | Nov. 18, 1952 |

##### FOREIGN PATENTS

|         |               |               |
|---------|---------------|---------------|
| 678,445 | Great Britain | Sept. 3, 1952 |
|---------|---------------|---------------|